

June 7, 1932.

F. L. ANTISELL ET AL

1,862,074

PRODUCTION OF COPPER CAKES AND SHEET BARS

Filed July 9, 1924

Fig. 1.



Fig. 2.



Fig. 3.



Fig. 4.



Fig. 5.

Fig. 6.

Frank L. Antisell  
Charles G. Mullineaux  
Inventors

By their attorney

Anthony Kline

## UNITED STATES PATENT OFFICE

FRANK L. ANTISELL, OF PERTH AMBOY, NEW JERSEY, AND CHARLES G. MULLINEAUX,  
OF ANSONIA, CONNECTICUT, ASSIGNEES TO ANACONDA COPPER MINING COMPANY,  
A CORPORATION OF MONTANA

## PRODUCTION OF COPPER CAKES AND SHEET BARS

Application filed July 9, 1924. Serial No. 724,983.

For the rolling of copper sheets and bars, the copper is first cast in what is called a "cake" of suitable size and shape to be conveniently handled and to fit the rolls, weighing around 225 pounds, oblong in plan and a few inches thick. What is called the standard cake, for example, is 14 x 17 x 2½ inches thick and is cast in this form with the 2½ inch dimension vertical and with a slight 10 taper at the sides to permit removal from the mold, usually of copper formed with a plunger.

The top face of such a cake takes a certain set or slight roughness in solidifying. Also 15 there is a certain amount of sweating on the sides and ends of the cake. This is the formation of fine particles like drops of copper on the otherwise smooth face of the cake, generally ascribed to the shrinkage of the cake at the outside while its center is still 20 molten and the exudation of fine drops of copper through to the surface.

In subsequent rolling of such cakes, the surface of the resulting sheets, is sometimes 25 bad because of the set or roughness on the top. Also the generally red sheen of the surface is marred by spots or zones of a yellowish color, familiar to experts and due apparently to oxidation.

We propose to avoid these disadvantages 30 by casting the cake differently. At the same time we have found in our improved cake certain other advantages referred to in detail hereinafter.

The accompanying drawing illustrates an 35 embodiment of the invention.

Fig. 1 is a side elevation of the cake in the cast position;

Fig. 2 is an edge elevation of the same;

Fig. 3 is a plan thereof;

Fig. 4 is a diagram illustrating the rolling of a sheet bar.

Figs. 5 and 6 are respectively a cross-section and a longitudinal section of the mold

40 filled with the cast copper.

We propose to cast the cake with its ends at the top and bottom in copper molds with the taper necessary for easy removal. This will produce a cake as shown with smooth sides

45 1 and edges 2 and a smooth lower end face 3,

and an upper end face 4 having the set or roughness involved in the solidifying of the casting.

We have found after considerable experimentation that cakes cast in this way can be 55 produced without sweating on the sides and edges. In practice we have made such cakes 16 inches long by 10 inches wide at the narrow end and about 4½ inches thick, with a taper on the sides and the edges of about 60 ¾ths of an inch, casting the metal at the usual temperatures and obtaining smooth sides and edges without any sweating.

Such a cake when rolled into a sheet bar 5 65 (Fig. 4) has a uniform surface without any of the yellowish spots that have appeared on such bars rolled from the standard cakes. In bars and plates rolled from standard cakes 70 such yellowish spots have apparently shown an inferior resistance to corrosion. They are 75 probably due to segregation of impurities in the top of the standard cake. Such impurities set up galvanic action with the copper which hastens corrosion by the well known phenomena of "local action." With bars and plates rolled from our improved cake there is a noticeable improvement in resistance to corrosion.

There is also a very great saving in scrap 80 for two reasons. First, the face of the new cake constitutes the rear end of the bar or sheet which is rolled. An irregularity on this end means a comparatively small cropping 6. The forward end is drawn out to a 85 tapering shape requiring a comparatively short cropping 7.

The second advantage over the standard 90 cake is that the new cake can be rolled with the aid of universal rolls. We have illustrated diagrammatically horizontal rolls 8 90 for the top and bottom faces and vertical rolls 9 for the side edges of the bar. The use of such edge rolls is made possible by the smoothness of the edges 2 of the new cake 95 and their freedom from sweating or other irregularity. The consequence is that no cropping of the bar 5 is required along its sides. With the standard cake above described, the sides have been so rough that a 100 universal mill could not well be used and the

rolled product has been both wavy and rough at the sides requiring cropping at both sides and both ends in order to secure a rectangular product.

5 It has also been proposed to cast cakes of a certain size for special sheets with a long narrow edge uppermost; but in rolling, this set edge has prevented the use of edge rolls and resulted in a rolled bar with one edge very 10 rough and irregular and the other wavy so that it had to be cropped as well as the ends. Such cakes were also badly sweated on their sides and ends. In our experiments, we have 15 found that such sweating is apparently due to the comparatively slight depth of the metal in the mold. From the depth of the standard cake, about 4 inches, up to about 7 or 8 inches, the sweating occurs in substantial extent. Above 8 inches the sweating 20 either disappears or is much reduced, and at about 12 or 14 inches depth it generally disappears entirely.

While we cannot say with certainty that it is so, we think the cause of the sweating 25 may lie in the difference in the depth and the freezing curve of the copper and its eutectoid in the two cases of a comparatively shallow and a comparatively deep casting.

In rolling copper longitudinally there is 30 incidentally a lateral flow which increases the width from 5 to 10%, and irregularly where edge rolls are not used to rectify it; the crop with these old style cakes has been approximately seven times the quantity necessary 35 with the new cake herein described.

The discussion above is based on the use of refined copper containing say 99.95% copper and 0.04% oxygen. The invention, however, is applicable with advantage to copper 40 of other degrees of purity.

The cakes referred to are to be distinguished from copper billets. These are generally round or square cross-section shapes from 2½ to 8 inches by about 42 inches long 45 and are used for fabricating into seamless tubing or bus bars of similar square sections made by the drawing process. Such billets are cast endwise in long molds which are usually accurately machined, the shrinkage 50 of the billet being depended on to release it from the mold.

The cakes of the present invention are cast in molds of copper, the interior surfaces of 55 which are formed by means of tapered plungers presenting faces which are sufficiently smooth for the subsequent rolling operation on the cakes, but which are not smooth enough to permit the removal of the cakes except with the aid of the tapered shape. 60 Such a mold is indicated in Figs. 5 and 6 with side walls 10, end walls 11 and bottom 12, the top being open for pouring in the metal. The taper of the side and end walls is sufficient to permit removal of the cake 65 without splitting the mold, and the integral

construction avoids the occurrence of the cracks in the mold which would form fins on the corners of the cake and would interfere with the subsequent rolling operations.

Though we have described with great particularity of detail certain embodiments of our invention, yet it is not to be understood therefrom that the invention is restricted to the particular embodiments disclosed. Various modifications may be made by those skilled in the art without departure from the invention as defined in the following claims.

What we claim is:

1. A copper cake of the character described for rolling into sheets and sheet bars, cast 80 endwise in tapered form so that its upper end constitutes the set face of the copper and its sides and edges are smooth, said cake being approximately 10 x 16 x 4½ inches.

2. A copper cake of the character described for rolling into sheets and sheet bars cast endwise in tapered form so that its upper end constitutes the set face of the copper and its sides and edges are smooth, the width, length and thickness of such cakes being substantially in the ratio of 10 x 16 x 4½.

3. The method of producing a copper sheet bar which includes in combination the following steps,—casting a cake with certain faces and edges in contact with the sides of a tapered one-piece mold which produces smooth surfaces on said faces and edges and rolling said cake out into a bar with rolls engaging said smooth surfaces.

4. The method of producing a copper sheet bar which includes in combination the following steps,—casting a cake with certain faces and edges in contact with the sides of a one-piece copper mold having its inner faces formed by a tapered plunger so as to produce smooth surfaces on said faces and edges and rolling said cake out into a bar with rolls engaging said smooth surfaces.

In witness whereof, we have hereunto signed our names.

FRANK L. ANTISELL.

CHARLES G. MULLINEAUX.

70

75

85

90

95

100

105

110

115

120

125

130